

Nov. 26, 1963

M. O. HOLOWATY ET AL.

3,112,212

## NON-SKID METAL SHEETS

Filed Dec. 3, 1959



Inverton's  
Michael O. Holoway  
Edmund S. Madryk  
with § Marshall  
ATTORNEYS

## 1

3,112,212

## NON-SKID METAL SHEETS

Michael O. Holowaty, Gary, Ind., and Edmund S. Madrzyk, Lansing, Ill., assignors to Inland Steel Company, Chicago, Ill., a corporation of Delaware

Filed Dec. 3, 1959, Ser. No. 857,018  
4 Claims. (Cl. 117—22)

This invention relates to novel methods of applying to the surface of metal sheets or strips abrasive particles or grit so as to render said metal sheets or strips resistive to slippage and skidding.

A method for applying the abrasive particles to the base metal is accomplished where the abrasive particles, such as silicon carbide of desired consistency and particle size, are suspended in a liquid metal carrier consisting of aluminum-zinc or aluminum-zinc-magnesium, the temperature of these alloys being in a range of 1250° F. to 1350° F. When the silicon carbide particles are suspended therein this carrier film abrasive particle combination may then be applied to the sheets while the base metal sheets are either hot or cold. In order to accomplish the suspension of the abrasive particles in the carrier metal it may be necessary to adjust the specific gravity of the carrier metal so as to permit the abrasive particles such as silicon carbide to be suspended therein. Once the base metal has been coated with the abrasive carrying alloy the resultant combination is submitted to quenching or gradual cooling as either may be desired to enable the alloy to adhere to the base metal.

This liquid alloy-abrasive particle suspension may also be processed into a shot-like product which is applied to the surface of the base metal strip in solid form and then melted in a suitable melting apparatus after the shot-like material has been applied to the base metal strip. The shot-like coating of the base metal may be done in a uniform manner covering the entire sheet or strip or the base metal may be spot coated at localized areas on the surface of said base according to a preferred design. The sheet or strip so coated after the melting process can be permitted to cool as desired to enable the coating metal to adhere to the base metal.

In the accompanying diagrammatic drawing:

FIGURE 1 is a schematic illustration of an embodiment of a method in accordance with the present invention; and

FIGURE 2 is a schematic illustration of a second embodiment of a method in accordance with the present invention.

Referring to FIGURE 1, in the embodiment of the method illustrated therein, abrasive particles are suspended in a molten alloy of the particular composition described above, and the molten alloy containing the suspended abrasive particles is formed into shot by conventional shotting methods, well-known to those skilled in the art. The resultant shot 51 is stored in a hopper 50 which distributes shot 51 onto the upper surface 57 of a continuous strip of flat metal base material 52. Flat metal base 52 containing shot 51 applied to the upper surface thereof then passes through a furnace 55 for melting the shot and fusing the alloy to upper surface 57 of base 52. If desired, before passing through furnace 55, base 52, containing shot 51 thereupon, may be passed through a pair of pressure rolls 53, 54 which exert just enough pressure to slightly fix the shot particles to upper surface 57 of

## 2

base strip 52. After melting of the shot and fusion of the alloy, strip 52 passes through a cooling zone 56 and from there to shearing means indicated generally at 59 for dividing continuous strip 52 into a plurality of sheets of relatively shorter length.

Referring to FIGURE 2, the embodiment of method illustrated therein provides a bath 60 composed of a molten alloy having a composition as described above and having abrasive particles suspended therein. A continuous flat metal base strip 52 passes downwardly into bath 60 around a bath roller 61 and then upwardly out of the bath. Also located in bath 60 is a roller scraper 62. A coating of molten alloy containing abrasive particles suspended therein is applied to both surfaces of strip 52 as it passes through the bath 60. Scraping means 63, located just above bath 60 for removing said coating from one surface 68 of strip 52, may be provided, if desired. As the coated strip moves away from bath 60 the molten coating becomes fused to the surface of base strip 52. Coated base strip 52 then passes between a pair of conventional turn-over rolls 64, 65 and is then cut into shorter lengths by conventional shearing means indicated generally at 59. The strip containing the coating fused thereto may be allowed to cool naturally between scraping means 63 and shearing means 59, or artificial cooling means, of a conventional nature well-known to those skilled in the art, may be utilized between scraping means 63 and shearing means 59.

Thus in each embodiment of the method of the present invention, the abrasive particle is suspended in a molten alloy of the particular composition described above, and the alloy containing the suspended abrasive particle is applied to the surface of a flat metal base and fused thereto to produce a non-skid flat metal material comprising a base, an alloy fused to the base, and abrasive particles suspended in the alloy. The base, of course, has a melting point substantially higher than that of the carrier alloy, and a typical example of a metal base is steel sheet.

Typical abrasive particles include, in addition to the aforementioned silicon carbide, boron nitride, sand, and the like, all of said particles being in finely divided form.

While the above described methods constitute a preferred embodiment of this invention it is obvious that the invention may be otherwise embodied and practiced so that all modifications which fall within the scope of the following claims are understood to have been intended.

What is claimed is:

1. A method for producing non-skid flat metal material, said method comprising:
  - providing an alloy selected from the group consisting essentially of aluminum-zinc and aluminum-zinc-magnesium and having a specific gravity which will maintain abrasive particles suspended in the alloy when the latter is molten;
  - suspending said abrasive particles in said alloy;
  - applying said alloy in molten form, and containing said suspended abrasive particles, to the surface of a flat metal base;
  - fusing said alloy to the base;
  - and then cooling to produce non-skid flat metal material comprising a base, an alloy fused to said base, and abrasive particles suspended in said alloy.

2. A method as recited in claim 1 wherein: said abrasive particles are suspended in said alloy when the alloy is in molten form at a temperature between about 1250° F. and about 1350° F., and said alloy is then applied to said surface of said base.
3. A method for producing non-skid flat metal material, said method comprising:
- providing an alloy selected from the group consisting essentially of aluminum-zinc and aluminum-zinc-magnesium and having a specific gravity which will maintain abrasive particles suspended in the alloy when the latter is molten;
- suspending said abrasive particles in said alloy;
- forming said alloy containing said suspended abrasive particles into shot;
- applying said alloy in the form of said shot to the surface of a flat metal base;
- melting said shot after it has been applied to said base and fusing said alloy to said metal base;

5

and then cooling to produce non-skid flat metal material comprising a base, an alloy fused to said base, and abrasive particles suspended in said alloy.

4. A method as recited in claim 3 wherein: said base is spot coated with said shot at localized areas on the surface of said base.

## References Cited in the file of this patent

## UNITED STATES PATENTS

|           |                   |       |                |
|-----------|-------------------|-------|----------------|
| 1,536,524 | Pfersdorff        | ----- | May 5, 1925    |
| 1,686,150 | Fink et al.       | ----- | Oct. 2, 1928   |
| 2,032,694 | Gertler           | ----- | Mar. 3, 1936   |
| 2,559,279 | Charles           | ----- | July 3, 1951   |
| 2,674,542 | Alexander         | ----- | Apr. 6, 1954   |
| 2,775,531 | Montgomery et al. | ----- | Dec. 25, 1956  |
| 2,853,401 | Mackin et al.     | ----- | Sept. 23, 1958 |
| 2,964,419 | Link et al.       | ----- | Dec. 13, 1960  |
| 2,998,322 | Strate            | ----- | Aug. 29, 1961  |